

June 3, 1969

R. C. MILLIKAN

3,448,320

ELECTRIC LAMP AND METHOD OF MANUFACTURE

Filed Dec. 15, 1966



Inventor:  
Roger C. Millikan,  
by John F. Ahern  
His Attorney.

1

3,448,320

**ELECTRIC LAMP AND METHOD OF  
MANUFACTURE**

Roger C. Millikan, Schenectady, N.Y., assignor to  
General Electric Company, a corporation of New  
York

Filed Dec. 15, 1966, Ser. No. 601,930  
Int. Cl. H01k 1/38, 19/50, 5/48

U.S. CL. 313—315

10 Claims

**ABSTRACT OF THE DISCLOSURE**

Incandescent lamps having incandescent filaments sealed through the exterior wall of a quartz envelope and making an intimate hermetic bond thereto are formed by passing the incandescent filament through a tubulation-type aperture therein, heating the wire to an elevated temperature, flushing the wire and the tubulation with a volume of inert gas sufficient to protect the incandescent filament against contamination from thermal decomposition products of the quartz tube and heating the quartz tube and the wire until the tube collapses about the wire to form an hermetic seal therebetween and in the absence of any intervening substance.

This application discloses improved electric lamps and similar structures utilizing an incandescent filament and is more specifically directed to such a structure in which a very thin filament is directly sealed through the ends of a quartz tubulation. This sealing is accomplished by carefully controlling the diameter of the wire, the temperature of the wire and the quartz during sealing, and the ambient atmosphere within which the seal is made to produce an intimate bonding of the quartz to the incandescent filament by a seal which does not crack, craze, or separate during or after operation of the device at temperatures up to 1000° C.

This application is related to my copending concurrently filed application, Ser. No. 601,927, and the copending concurrently filed application of R. C. Millikan and L. A. Osburg, Ser. No. 601,927.

For many years the incandescent lamp has been the standard source of illumination, particularly for low power applications wherein color rendition is of great importance. Unfortunately, theoretical and practical maximum efficiencies of an incandescent lamp are relatively low, since the radiation from an incandescent filament is substantially black-body radiation and only a minor fraction thereof lies within the visible spectrum, the greatest proportion thereof being dissipated in the form of heat. Because of its relatively small size and low cost, however, the incandescent lamp has been able to compete effectively with other light sources for the low voltage consumer market. Research efforts to improve the efficiency of incandescent lamps has nevertheless continued. The presently commercially available best example of the highest efficiency presently obtainable in incandescent lamp filaments is typically represented by lamps known as the Quartzline type of incandescent lamp such as those disclosed by Fridrich et al., U.S. Patent No. 2,883,571, issued Apr. 21, 1959, and assigned to the General Electric Company, and by other related patents disclosing and claiming improvements thereupon.

In general, Quartzline type lamps are characterized by a thin cylindrical tube of quartz having a relatively long, longitudinal concentric tungsten filament, the diameter of which constitutes a substantial fraction of the diameter of the inner wall of the quartz tube, whereby the inner wall of the quartz envelope is operated at a relatively high temperature. Degeneration of the hot tungsten

2

filament is prevented by the presence, within the quartz envelope, of a low partial pressure of iodine in a buffer gas which, at the operating temperature of the filament is responsible for the presence of a regenerative iodine cycle which prevents accumulation of tungsten from the filament upon the interior bulb walls. This accumulation has the dual deleterious effect of lowering the transmissivity of the walls and causing the tungsten filament to be dissipated. Utilizing the iodine cycle, the tungsten on the bulb walls is recombined with iodine to form a tungsten-iodine compound which migrates to the hot filament, is decomposed and causes the tungsten to be redeposited upon the filament.

Although lamps such as those described hereinbefore are among the most efficient and long-lived incandescent lamps available today and are highly effective in competition with other light sources, the necessary steps which must be taken in order to achieve the high efficiencies and long life characteristic of the lamps result in production costs which are highly undesirable for commercial manufacture of such lamps. One such cost relates to the expensive double-welding process whereby the filament is welded to a foil of molybdenum which is then sealed through the quartz. A lead wire having mechanical strength and durability must be welded to the opposite end of the molybdenum foil, thus requiring four welds and the use of a fragile molybdenum foil in fabrication of the lamps. Additionally, such structure requires the utilization of an inordinately large quantity of quartz which is uneconomical.

Accordingly, it is an object of the present invention to provide high efficiency incandescent lamps wherein a simple, economical, and effective means is provided for sealing the incandescent filament through the quartz wall at the end thereof.

It is another object of the present invention to provide a method for simply and effectively directly sealing an incandescent filament through the end of a quartz envelope in an hermetic and mechanically strong seal which will not crack or craze under operating conditions.

Still another object of the invention is to provide lamps having improved quartz to refractory metal seals.

In accord with the present invention, I provide incandescent lamps having a quartz or quartz-like envelope and a refractory incandescent filament therein, wherein the incandescent filament is directly sealed through the wall of the quartz envelope without any intermediate element to facilitate the seal. Such seals directly between the incandescent filament and the quartz envelope may readily be made by keeping the diameter of the wire constituting the filament at a value of less than 0.004 inch, by out-gassing the filament wire prior to and during sealing to preclude the presence of any adsorbed gas thereupon and by continuously flushing the filament and the quartz during sealing to preclude the presence of any molecular or gaseous impurities evolved from either during heating to be interposed between the quartz and metal in the final seal.

The novel features believed characteristic of the present invention are set forth in the appended claims. The invention itself both as to its preferred embodiments and mode of operation, together with further objects and advantages thereof may best be understood with reference to the following detailed description taken in connection with the appended drawing in which:

FIGURE 1 is a vertical cross-sectional view of an incandescent lamp constructed in accord with the present invention, and

FIGURE 2 is a vertical cross-sectional view of an alternative embodiment of the device of FIGURE 1.

Since quartz was first used as an incandescent lamp envelope those skilled in the art have been attempting to make seals through quartz envelopes to incandescent

lamp filament by a variety of methods. Since quartz has a temperature coefficient of expansion that is exceedingly different from that of most metals and particularly different from that of refractory metals, this has presented a very serious problem in instances in which the area of the final seal is to be subjected to high temperature. As described hereinbefore, the most effective and efficient incandescent lamps now utilize a configuration wherein the quartz including that portion thereof which constitutes the seal is operated at a substantially higher than room temperature during normal operation. For this reason the difference in thermal coefficients of expansion, if not in some way compensated for or otherwise avoided, results in seals which, when subjected to large temperature changes, degenerate by a separation of the metal from the quartz, resulting in the loss of hermetic sealing between the wire and the quartz. Due to the fragility of most incandescent filaments no attempt has ever been made to directly seal the incandescent filament through the quartz of incandescent lamp envelopes. Instead, workers in the prior art have generally relied upon the passage of the current carrying member through the quartz to effectuate a seal by virtue of an intermediate member which is connected to the incandescent filament on one end thereof and to the supporting lead at the other end thereof. As is mentioned hereinbefore, this is a costly, complicated and self-defeating approach since it requires four welds and an intermediate body which may have a number of configurations but which in general is difficult to work with and very expensive. Examples of the expedients taken in the prior art are as shown, for example, in the aforementioned Fridrich patent in which a refractory support member having a flattened end is utilized to form the seal and the filament is welded to the flattened end of the lead member.

Another approach is that set forth in Patent 1,271,245 to VonRecklinghausen in which one or more members having a portion thereof which is very small in one transverse dimension but very large in another transverse dimension, as for example by flattening a portion of the wire into a thin ribbon thus preserving the same total cross-section but maintaining at least one dimension thereof very small, attempts to seek release from the differential expansion problem. In yet another attempt sought by the prior art, Patent No. 1,922,536, Ericson sets forth an extremely complicated method whereby a thin intermediate member is sealed in a quartz tubulation and connected to at either end thereof to provide a seal. In yet another attempt to solve the differential expansion problem Patents Nos. 1,489,009 and 1,118,812 to Reynolds and Sand and Reynolds respectively, utilize a tungsten lead member with a lead coating thereupon which is sealed through a quartz member. In yet another attempt to solve through a quartz differential expansion problem, in Patent No. 832,302 to Ernst, an intermediate element comprising a thin tungsten wire sealed through a thin glass tubulation is provided for incorporation in a glass, hermetically sealed device by connecting a thin tungsten wire within a cylindrical glass tubulation and connecting the tubulation to a vacuum pump. Then, while the vacuum pump exhausts the tubulation to a low pressure, selected portions of the tubulations are heated so as to cause them to collapse around the glass and form a tight seal thereabout. Either end of the collapsed portion of the glass is then cut to provide an element comprising a thin piece of glass having a thin tungsten wire hermetically sealed thereto. This piece of glass may then be used as a seal in a glass envelope for a variety of uses.

In accord with the present invention I avoid the extremely complicated and expensive expedients of the prior art by the simple approach of directly sealing the filament through a quartz envelope under such conditions as to form a strong, temperature-resistant seal which does not degrade or separate from the wire during operation at temperatures even as high as 1000° C. for example.

The structure of the present invention is illustrated in one embodiment in FIGURE 1 of the drawing in which hermetically sealed envelope 1 includes a hollow cylindrical portion 2 with a closed tubular shaped end portion 3 at either end thereof. An incandescent filament 4 is located concentrically along the axis of envelope 1 and passes completely through end portions 3 thereof without interruption or termination. As illustrated in FIGURE 1, the coil of the filament is terminated and the filament assumes a configuration of a straight wire upon emerging from envelope 1. This is optional, however, and the filament may emerge from envelope 1 in the same configuration as it exists within cylindrical portion 2 thereof or as a straight wire as illustrated in FIGURE 1. Additionally, although the filament is illustrated in FIGURE 1 as being a single wire and including a single helical coil in the central portion thereof any conventional or convenient filament configuration as for example those set forth in the copending application of P. D. Johnson, Ser. No. 580,995, filed Sept. 21, 1966, the entire specification of which is incorporated herein by reference thereto, may be utilized provided that the elemental wire thereof from which the filament is fabricated meets the dimensional criteria set forth herein.

I find that an effective strong seal may be made between a tungsten filament and a quartz envelope if the elemental wire comprising the incandescent filament is less than 0.004" in diameter, if the wire is heated to a white heat prior to and during sealing to force the evolution therefrom of any adsorbed gasses, and if means are provided to remove all material ejected from the filament during the heating thereof and to prevent material ejected from the quartz from migrating to and contaminating the filament prior to or during sealing. The incandescent filament 4 may conveniently be of any refractory material suitable for operation at incandescent temperatures, as for example tungsten, molybdenum, rhenium, but for purposes of simplicity in this application will be referred to as a tungsten wire. I find that if the tungsten wire is 0.004" or less in cross-sectional diameter, the seal formed with quartz may be operated repeatedly and for many hours at a temperature up to 1000° C., for example, and repeatedly cooled back to room temperature without degradation of the seal. I believe this is possible due to the distribution of stresses along the radial and tangential directions of the circular cross-section of the wire is such that the difference between thermal coefficient of expansion and of the quartz and tungsten does not cause a separation between the two, provided the initial bond is between the two directly and there is no interposed impurity layer which tends to weaken the same. As a practical matter, I find that for the construction of useful commercial incandescent lamps a filament wire diameter of 0.0005" represents the practical low limit with which one can make lamps in accord with the present invention.

Prior workers in the art have attempted to form effective tungsten to quartz seals by deliberately forming upon the surface of the tungsten an oxide coating of several monolayers thickness or greater, which had the purpose of providing a resilient means for taking up for differential expansion. To the contrary, I find that such interposed oxide layers are extremely deleterious and tend only to form an easy source of cleavage between the tungsten and quartz upon differential expansion or contraction. Accordingly, I provide my tungsten filament in a substantially unoxidized state by conventional prior heat treatment and out-gassing the heat and filament during sealing to a temperature of from 1750 to 2200° C., which is a white heat, to remove any surface adsorbed gasses thereon.

Although the heating of the tungsten filament may be accomplished by passing an electric current therethrough, I prefer to heat the filament by the passage of a flow of extremely hot gas longitudinally along the filament during sealing. This has the added advantage of not only heating

the filament but also removing therefrom any impurities evolved by heating and serving as a buffer to prevent the deposition thereupon of any impurities evolved from the quartz. The gas utilized to heat the filament is preferably a gas which does not react with quartz or tungsten as for example nitrogen or one of the noble gasses. The pressure at which the flushing gas is utilized may be any value in excess of 1 mm. of mercury pressure although in general as the velocity of the flushing gas decreases it is preferred that the pressure of the gas increases. This is because, as stated hereinbefore, one essential function of the flushing gas is to shield the tungsten filament from any impurities evolved from the quartz during heating in sealing.

When quartz is heated to its softening point to the extent that it can be expected to contract around, and seal with, a tungsten filament, as for example, a temperature of 1750 to 2200° water vapor is evolved therefrom. Water vapor in the presence of a hot tungsten filament can set up a deleterious cycle whereby the water molecules migrate to the tungsten, are decomposed thereat, forming tungsten oxide and a tungsten compound which migrates back to the quartz, removing tungsten from the filament. This cycle is very detrimental in the formation of tungsten filaments and, therefore, it is exceedingly important that, when the quartz is heated in the formation of the seal the water vapor evolved from the quartz be prevented from reaching the tungsten filament. This may be achieved by the passage of high velocity gas between the two even at reduced pressures of for example 1 mm. of mercury of the flushing gas. The same objectives may, however, be achieved at lower flushing velocities or even for brief periods of time at which the velocity of the gas between the quartz and the tungsten is essentially zero, as for example, just prior to making of the final seal in a closed system, unless some other orifice is provided to allow for a path for flushing of the gas. In this instance, it is highly desirable that a very high pressure of a high molecular weight inert or noble gas such as argon or krypton be provided in order that the mean free path of the water molecules be very short as compared with the distance between the quartz and the tungsten.

As an example of a pressure distance relationship which satisfies this mean free path requirement it is sufficient, utilizing a 0.002" wire in a 0.040" inside diameter quartz tubulation that the pressure of the flushing gas or the interposed gas, even without flushing, be approximately 10 mm. of mercury. This yields a mean free path of the water molecule of approximately 0.0005", which clearly makes it highly improbable that any water molecule may reach the tungsten filament.

By virtue of the foregoing discussion, it should be readily understood that it is not practical or desirable to attempt to form seals between tungsten and quartz by this or any other method wherein the substitution of a vacuum environment for an inert gas environment (often considered equivalent in related arts) is made. This is because, if a vacuum is established within the distance between the filament and the quartz and the quartz is heated to cause the softening thereof, under vacuum conditions the mean free path of water vapor evolved from the quartz becomes exceedingly long and the probability of water reaching the tungsten filament and setting up a water cycle, which causes the deposition of the layer of tungsten oxide upon the tungsten filament, is very great. Accordingly the last thing to be considered in the formation of such seals would be the evacuation of the region between the tungsten and the quartz during sealing.

In forming lamps in accord with the present invention, it is convenient to take a section of quartz tubing as illustrated in FIGURE 1 of the drawing, having an outside diameter of approximately 10 mm. and an inside diameter of approximately 8 mm. with a "necked down" end section on either end thereof having an outside diameter of approximately 8 mm. and an inside diameter of approximately 2 mm. Conveniently, the inside diameter of the

constricted end portion of at least one of the ends of the quartz tube is made large enough to accommodate the outside diameter of the configuration of the coil of filament 4. Since the filament need be inserted in only one end this requirement need be present at only the end from which the filament is inserted.

Also conveniently, the quartz tube may be provided with an exhaust-type tubulation at the center thereof for provision of a ready path of flushing for the second seal after the first seal is made and for evacuation or filling, as for example with low pressure iodine, of the enclosure within the envelope or raising or lowering of the pressure thereof, as desired. After sealing both ends and after whatever operation is desired to be performed through this tubulation is performed, the tubulation is closed off, leaving a nipple 5 which completes the hermetic sealing of the envelope. It is to be appreciated, however, that such a tubulation and remaining nipple are in accord with only one feature of the invention and the lamps in accord with the invention may be fabricated without such tubulation.

Assuming such a tubulation is present, fabrication of the lamp of FIGURE 1 may be as follows. The quartz tube, as described above, has a conveniently coiled or coiled-coil helical filament which may or may not have straightened ends but which, for convenience of description, will be assumed to have straightened ends as illustrated in FIGURE 1, is inserted thereinto through the larger diameter end portion 3 and the straightened end portion 6 is caused to emerge from the other end portion 3. The quartz tube is then placed in a suitable fixture and a jet of argon, for example, at a pressure of, for example 10 mm. of mercury is directed into the aperture within the first end 3 to cause the flushing of the entire interior of the envelope with argon gas. The flow of flushing gas and low internal pressure are maintained by any appropriate suction device. This gas is heated to an elevated temperature by external torching or other application of heat to the quartz so as to cause the temperature of the filament to be raised to a temperature of from 1750 to 2200° C. At temperatures below 1750° insufficient out-gassing and desorption of surface adsorbed gas particles is present and it is difficult to make good seals. At temperatures in excess of 2200° C. the effects upon the quartz envelope are such as to preclude its maintaining its structural rigidity. I have found that it is preferable, both from the point of view of forming optimum degassed tungsten surfaces and for maintaining the structural rigidity of the quartz during fusing, to cause the gas heating to provide a filament temperature of from 1800 to 2000° C. After the filament has reached this temperature, as measured by an optical pyrometer, the quartz is heated more intensely, which may for example be a second jet of high temperature gas directed thereabout, as for example from a peripheral nozzle located thereabout, or by an annular resistive heater encircling region 3, or by plasma torch or focussed laser heating to cause the temperature of the quartz to be raised above 2200° C., causing the quartz to collapse about the tungsten filament and form an hermetic seal therewith.

The quartz may be caused to collapse about the filament and seal thereto by applying a constrictive force thereto. Such a force may, for example, be supplied by pressure differential of, for example several pounds per square inch, caused by pumping the flushing gas out from the quartz envelope through the tubulation at nipple 5, as described above, so that the pressure within the envelope is slightly less than outside the envelope. Alternatively, the end 3 may be mechanically squeezed by any suitable means. After one end of envelope 1 has been sealed, the process is repeated with the other end, the high temperature gas which is injected into the restricted diameter end portion 3 escaping through the tubulation at the center of the tube to allow free flushing of the device. After the second end portion has collapsed about the tungsten filament to cause the formation of an

hermetic seal, the center tubulation is sealed off (after any desired filling or pressure change therethrough) leaving nipple 5, and the incandescent lamp fabrication is completed.

In accord with another embodiment of the present invention, substantially the same procedure is utilized, as described above, with the exception that no center tubulation is provided and the second seal is made at a higher pressure of inert gas, as for example, approximately 1 atmosphere, thus relying upon the high pressure of inert gas molecules in the vicinity of the filament and the quartz to which it is to be sealed to reduce the mean free path of water evolved from the quartz so as to preclude the presence of a water cycle and the deposition of tungsten oxide upon the tungsten filament.

In FIGURE 2 of the drawing there is illustrated a lamp constructed in accord with another embodiment of the invention. In FIGURE 2, the lamp comprises a cylindrical quartz member 10 having a central aperture 11 therein for the accommodation of a filament 12 which passes concentrically therethrough. At either end of opening 11, the quartz constituting cylinder 10 has been collapsed about filament 12, forming seal regions 13, which seals were made substantially as described with respect to the formation of the device of FIGURE 1. The respective ends of cylindrical quartz tubulation 10 include re-entrant openings 14, which are filled with an electrical contact-making and mechanically support-producing filling 15 of a suitable metal, as for example nickel, which is readily adaptable for making electrical contact to the emerging filament lead 16. The ends of the tubulation 10 are closed with metallic caps 17, which may conveniently be made of nickel and which are suitably soldered nickel inserts 15 within tubulation 10. Electrical contact to the lamp may then be made to end caps 17 to provide for the flow of electric current through filament 12 to produce incandescence therein and the subsequent emission of suitable and useful light. The structural characteristics and suitable methods for forming the filling 15 in re-entrant portions 14 of envelope 10 are described in greater detail and claimed in the copending, concurrently filed application of R. C. Millikan and L. A. Osburg, application Ser. No. 601,927, which is assigned to the assignee of the present invention.

In describing the formation of the lamps of the present invention, I have indicated a preference for nonreactive gasses as the medium for flushing the quartz tubulation and for heating the tungsten wire. Although this is the case, it is possible to form lamps in accord with the present invention using low pressure atmospheric air for these purposes. In this instance, provided the pressure of the air is low enough, as for example from 10 to 100 mm. of mercury, substantially little oxide is allowed to form upon the surface of the tungsten filament. Even if a very small amount of oxide does form as for example a monolayer, the solubility of tungsten oxide in quartz is sufficient so that a very small amount of oxide may be absorbed within the quartz immediately upon making contact thereto, thus allowing the quartz to make intimate contact with the metallic tungsten of the filament which facilitates the formation of good seals in accord with the present invention.

From the foregoing it will be evident that I have disclosed improved incandescent lamps utilizing refractory metal filaments which are simple, inexpensive and easy to manufacture and wherein a refractory metal filament having a metal wire diameter of not to exceed 0.004" is directly sealed through a quartz envelope wall without the interposition of any intermediate member or any welding thereto. This sealing is accomplished by the heating of the refractory filament to a white heat of 1750° to 2200° C. and a flushing with hot gas to remove evolved impurities or, in the alternative, the presence of a high pressure gas to see that impurities evolved from either the tungsten or the quartz do not return to the

75 tungsten to cause the formation of deleterious coatings thereupon.

One lamp in accord with the invention was made with a 3" long quartz tube of 0.250" O.D. and 0.150 I.D. and an exhaust tubulation of 0.100 O.D. at the longitudinal center thereof. A 0.002" diameter tungsten wire having a helical coil having a diameter of 0.050" and a length of 1" was suspended along the longitudinal axis of the quartz tube and extending along its entire length. One end of the tube was closed by an O ring and an end clamp and the other end was connected temporarily to a source of dry nitrogen at a pressure of 10 mm. of Hg. A mechanical fore pump was connected to the exhaust tubulation and operated to draw the nitrogen through one end of the quartz tube at a flow rate equivalent to 1 cc. per second at conditions of standard temperature and pressure. Heat was applied to the quartz wall about 1" from the end with a pair of oxyhydrogen torches at a rate sufficiently slow to allow the tungsten wire to come to a temperature of 1800° C. before the quartz was deformed. This was accomplished by a 2 minute heating cycle. After 2 minutes of heating the softened quartz was drawn by the pressure differential into contact with the tungsten wire and the seal was made. The procedure 20 was repeated with the nitrogen source connected to the other end to produce the second seal. The exhaust tubulation was then heated until it softened and sealed over completely. The resultant lamp was as is illustrated in FIGURE 1.

30 Although the desirability for the improvements achieved by the present invention are of particular importance in Quartzline type incandescent lamps utilizing iodine or other halogen regenerative cycle, it should be appreciated that the invention set forth herein is applicable to the generalized structure of quartz and quartz-like lamp envelopes and is not limited to lamp envelopes containing any particular gaseous filling. Similarly although for convenience the invention has been described in connection with pure quartz envelopes it should be appreciated that the invention may be practiced with any light-transmissive vitreous predominantly silica material as for example, Vycor (95% SiO) which is predominantly silica and has a quartz-like low thermal coefficient of expansion which renders the passage of metallic electrical lead wires therethrough a problem of such magnitude as is described herein and which may be solved by the principles of the present invention.

While the invention has been described herein with respect to specific embodiments and examples thereof it will be appreciated that many modifications and changes will readily occur to those skilled in the art. Accordingly I intend by the appended claims to cover all such modifications and changes as fall within the true spirit and scope of the invention.

50 55 What I claim as new and desire to secure by Letters Patent of the United States is:

1. An incandescent lamp comprising:

(a) an hermetically sealed envelope of a vitreous light-transmissive high silica material having a low quartz-like coefficient of thermal expansion;

(b) a refractory metallic wire incandescable filament supported within said envelope and sealed directly through said envelope without interruption or deformation and emerging as a current conductor exterior of the hermetically sealed portion of said envelope;

(b<sub>1</sub>) said filament being sealed through said envelope by intimate contact between said metal and the material of said envelope in the absence of intervening substance.

60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9

4. The lamp of claim 2 wherein a lamp envelope is quartz.

5. The lamp of claim 3 wherein the lamp envelope is Vycor.

6. The lamp of claim 3 wherein the lamp envelope is in the form of an elongated cylindrical tube and said filament is in the form of an axial coiled helix, said helix occupying a substantial portion of the interior cross-sectional area of said tube.

7. The method of making an incandescent lamp which comprises:

(a) providing an envelope of a vitreous light-transmissive high silica material having a low quartz-like coefficient of thermal expansion having at least one constricted end portion with an aperture therein;

(b) disposing a refractory metallic incandescent filament within said envelope with an end of said filament extending through said aperture;

(c) heating said filament to a temperature of approximately 1750° C. to 2200° C. in an inert gas atmosphere to outgas the surface thereof, said gas being present in pressures sufficient to prevent contamination of the surface of said filament by thermal decomposition products of said high silica material; and

(d) heating said constricted end portion above the softening point thereof to cause the envelope end

to constrict about said filament while maintaining said filament at said elevated temperature to form an intimate, hermetic seal therewith.

8. The method of claim 7 wherein said filament is heated by a flow of heated inert gas at a pressure of in excess of 10 mm. of mercury.

9. The method of claim 8 wherein the inert gas is argon at a pressure of 10 mm. of mercury to one atmosphere.

10. The method of claim 8 wherein the inert gas is pure dry nitrogen at a pressure of 10 mm. of mercury to one atmosphere.

#### References Cited

##### UNITED STATES PATENTS

|    |           |         |             |       |           |
|----|-----------|---------|-------------|-------|-----------|
| 15 | 1,293,594 | 2/1919  | Willey      | ----- | 313—318 X |
|    | 2,273,437 | 2/1942  | Dunn        | ----- | 313—318 X |
|    | 2,276,218 | 3/1942  | Lemmens     | ----- | 313—318 X |
|    | 3,040,204 | 6/1962  | Belknap     | ----- | 313—274 X |
| 20 | 3,080,497 | 3/1963  | Noel et al. | ----- | 313—271 X |
|    | 3,211,943 | 10/1965 | Cardwell    | ----- | 313—315   |

JAMES W. LAWRENCE, Primary Examiner.

RAYMOND F. HOSSFELD, Assistant Examiner.

25 U.S. Cl. X.R.

29—25.15; 313—174, 274, 318, 331